

## UNITED STATES PATENT OFFICE

2,287,948

## INDIUM PLATING

Clarence F. Smart, Pontiac, Mich., assignor to  
General Motors Corporation, Detroit, Mich., a  
corporation of DelawareNo Drawing. Application December 16, 1938,  
Serial No. 246,064

1 Claim. (Cl. 204—45)

This invention relates to the electro-deposition of indium and has particular reference to a process and bath for plating indium by electro-deposition.

The primary object of my invention is to provide a new and improved bath and process for the electro-deposition of indium having certain advantages over baths and processes heretofore proposed for this purpose. Other objects and advantages will become apparent from the detailed description.

The bath of the present invention is one that has exceedingly good throwing power, is one of good efficiency, and one that is easy to operate and control. The allowable ranges of current densities, voltages, etc., for good deposits are quite broad. The bath is easy to make up in the first place and is free of the danger of HCN fumes, such as might occur in the making up of a cyanide bath unless the operations are performed under a well ventilated hood, etc. The bath of my invention has little or no tendency to dissolve such metals as iron, nickel, cadmium, silver and copper and thus is not subject to contamination by these metals; in addition, it shows no tendency for the indium to separate on long standing, remaining clear and free from sludge. Deposits plated by the use of my bath and process are smooth, adherent and free from the dark smudge sometimes present in deposits from cyanide baths. The indium may be readily recovered from the bath.

I have discovered that a bath comprising indium, dextrose, an alkali, such as sodium hydroxide or potassium hydroxide, and water has certain advantages in the electro-deposition of indium over other baths of which I am aware. The indium content may be from about one to six ounces per gallon of water, dextrose may be approximately half the indium content, but preferably not under about one ounce per gallon, and sodium hydroxide or potassium hydroxide from about six to twelve ounces per gallon. The sodium hydroxide is less expensive than the potassium hydroxide and is, therefore, preferred. A preferred composition is approximately as follows: indium 4 oz. per gallon of water, dextrose 3 oz. per gallon of water, and sodium hydroxide 8 oz. per gallon of water.

The plating bath of my invention operates well at ordinary temperature of 70° F., also at higher temperatures up to 175° F. if desired, over a wide range of voltage and current density. Good, adherent, deposits of indium have been obtained with voltages from about 3 to 10, and

current densities from about 10 to 150 amperes per square foot of cathode area. At lower current densities the deposits are smoother than are those obtained with the higher current densities. 5 Inert anodes, such as carbon, for example, are employed.

The bath may be made by dissolving metallic indium in hydrochloric acid and to this solution adding a water solution of sodium hydroxide or 10 potassium hydroxide or the like to which dextrose has been added. The indium is first precipitated as white indium hydroxide and then in the presence of excess alkali and dextrose the indium redissolves leaving a clear solution. It is permissible to add the dextrose to either the 15 concentrated sodium hydroxide or potassium hydroxide solution, or to the concentrated solution of indium in acid, and to add either one of these to the other with stirring to dissolve the precipitate which first forms. After mixing the concentrated solutions, water is added in order to obtain the desired solution. The solutions should be cool before mixing, as at boiling temperatures the indium hydroxide precipitates and does not 20 redissolve. This reaction may be made use of if it is desired to recover the indium from the bath for any reason. For example, it may be desirable to recover the indium from a partially depleted bath with too low indium content for satisfactory current efficiency. By heating the bath to a boiling temperature the indium is completely precipitated as indium hydroxide and may be separated as by filtration, or by settling and decantation. The precipitate may be redissolved 25 in acid and made into a new plating bath if desired.

In place of hydrochloric acid the indium may be dissolved in other acids such, for example, as sulphuric acid or nitric acid. I prefer the hydrochloric acid, however, as excess acid can be readily removed from the solution by boiling and because the hydrochloric acid is non-oxidizing to the dextrose. Soluble salts of indium may be used, if available, to dissolve directly in water 30 without acid.

By the use of my bath and process indium may be plated on metals of various kinds, as desired. My bath is especially desirable in plating bearings or bearing alloys to render the same corrosion resisting. Cadmium alloy bearings and copper-lead bearings may be readily plated with indium to provide a corrosion resisting coating thereon. The plated bearings may be heat treated at about 340° F. to cause the indium to 35 become diffused into the base metal.

While I have described a preferred embodiment of my invention, I am aware that many changes may be made and numerous details varied without departing from the principles of my invention and I do not desire to limit the patent granted for my invention except as necessitated by the prior art.

I claim:

A process for the electro-deposition of adherent deposits of indium comprising, passing an electric current through an electrolyte from an inert anode to a cathode under a voltage of from about three to ten volts and with a current den-

sity of about 10 to 150 amperes per square foot of cathode area; the electrolyte being free of at least substantially all cyanide and consisting of an aqueous solution of the following essential constituents in approximately the amounts given per gallon of water: a compound of indium in which the indium content is about one to six ounces, dextrose approximately half the indium content and at least one ounce, and sodium hydroxide from about six to twelve ounces; said electrolyte being maintained during operation at a temperature of about 70° F. to 175° F.

CLARENCE F. SMART.

2,287,948

2,287,948

2,287,948

2,287,948

2,287,948

2,287,948

2,287,948

2,287,948

2,287,948

2,287,948

2,287,948

2,287,948

2,287,948

2,287,948

2,287,948

2,287,948

2,287,948